

Dec. 4, 1962

G. A. FASOLD ET AL

3,066,793

FIRE AND WEATHER RESISTANT JACKETING

Filed March 17, 1958

2 Sheets-Sheet 1



**FIG. 1.**



**FIG. 2.**



**FIG. 3.**

INVENTORS.  
GEORGE ARTHUR FASOLD  
AND RALPH J. O'CONNOR,  
BY

*Allen Allen*

ATTORNEYS.

Dec. 4, 1962

G. A. FASOLD ETAL

3,066,793

FIRE AND WEATHER RESISTANT JACKETING

Filed March 17, 1958

2 Sheets-Sheet 2



**FIG. 6.**



**FIG. 5.**



INVENTOR,  
GEORGE ARTHUR FASOLD  
AND RALPH J. O'CONNOR,  
BY

*Allen Allen*

ATTORNEYS.

# United States Patent Office

3,066,793

Patented Dec. 4, 1962

1

3,066,793

**FIRE AND WEATHER RESISTANT JACKETING**  
George Arthur Fasold, Mount Healthy, and Ralph J. O'Connor, Glendale, Ohio, assignors to The Philip Carey Manufacturing Company, Cincinnati, Ohio, a corporation of Ohio

Filed Mar. 17, 1958, Ser. No. 721,709  
2 Claims. (Cl. 206—59)

Our invention relates to new and useful improvements in fire and weather resistant jacketing particularly for covering outdoor insulated pipe lines.

In industrial establishments there are often installations in which tanks in one building are connected by pipes with apparatus (pumps or the like) and other tanks in other buildings and it is highly desirable to provide jacketing for covering the insulation on the pipes. If these pipes are merely covered with ordinary asphalt saturated and coated felt or roofing material there is a tendency for a fire in one building to spread through combustion of the sheet material covering to the other building. This is a definite fire hazard.

In our new weather resistant jacketing it is our object to provide:

- (1) A sheet material which resists spread of flame and the dripping of asphalt which would otherwise propagate combustion.
- (2) A sheet material having a permanent white surface and long life and maximum efficiency.
- (3) A sheet material which will have weather resistant properties.

(4) A sheet material which is flexible and will not crack when applied over a small size pipe covering.

(5) A sheet material of high tensile strength.

(6) A sheet material reinforced so as to be very tough and resistant to tearing with the wire tying required in its application and attachment over pipe insulation.

The foregoing objectives we accomplish by the provision of a reinforced jacketing assembled in a particular manner as will hereinafter be described.

In the drawings which illustrate diagrammatically a preferred construction:

FIGURE 1 is a cross sectional view of a piece of insulated pipe with the preferred jacketing installed.

FIGURE 2 is an enlarged lengthwise sectional view as would appear along the lines 2—2 of FIGURE 1.

FIGURE 3 is a diagram illustrating a modified arrangement of fill threads applied to the jacketing during its manufacture.

In order to first explain where and how our new jacketing is used, reference may be made to FIGURE 1 in which 1 indicates a pipe for steam, hot water or other liquid. The insulation for the pipe is illustrated at 2 and it may be built up from blocks of asbestos and magnesia or formed from precast arcuate segments applied to the pipe in segments which are bound together.

At 3 we have illustrated the jacketing material forming the subject matter of our invention the sheet material being wrapped around the insulation and overlapped as indicated at 4 with a wire 5 holding the jacket in place, the wire being cut off and crimped or twisted into a binding series of loops as indicated at 6.

In FIGURE 2 the construction of the jacketing material is indicated. The inside ply indicated at 7 is a sheet of saturated asbestos felt. The saturant used preferably has a penetration ASTM D5 @ 77° F. 90 to 125.

Applied to the outer surface of the felt is a film 8 of

2

asphalt adhesive. This asphalt adhesive has preferably the following characteristics:

|                                    |            |
|------------------------------------|------------|
| Softening point (ring & ball)----- | 215 to 235 |
| ASTM D-36 @ 77° F-----             | 17 to 22   |
| ASTM D-36 @ 32° F-----             | 12 to 16   |
| ASTM D-36 @ 115° F-----            | 30 to 40   |

Flash point ASTM D-92 over 500° F.

Blend of Midcontinent crude oxidized.

10 Softening point and penetration can vary 25% either way.

Within the coating of adhesive and penetrating into it there is a layer of 1/2 in. glass scrim 9 formed with warp threads extending crosswise of the sheet and being normally unwoven in the scrim structure. Surrounding the jacket and forming the outer ply is a sheet of preferably 11 lb. asbestos felt 10 having a white outer surface which preferably is treated with a parafinaceous ingredient in the beater so that the white outer surface is substantially permanent.

15 It should be understood that in the glass scrim which we ordinarily incorporate in our jacketing during its manufacture in sheet form the warp threads which extend lengthwise of the sheet are primarily of importance only because they carry the fill threads which are laid across them. The fill threads preferably of glass fibers extend crosswise of the sheet and are of great importance in building up the toughness of the material and resistance to tearing as when the wires 5 are bound around the jacketing material to hold it in place.

20 In FIGURE 3 we have illustrated diagrammatically an arrangement by which the glass threads 9a which form the fill threads of the reinforcement are ejected by air from a series of nozzles arranged side by side at spaced intervals lengthwise of the sheet which eject the threads in a series 25 of swirling loops, 9a, as the sheet moves along. These loops extend widthwise of the sheet and overlap and are held in the coating of adhesive. The top ply 10 of asbestos felt is then applied and the combined plies are 30 then rolled up in rolls.

25 That the fill threads of glass fibers extend crosswise of the rolls is substantially preferable because when pieces are cut from the rolls of finished jacketing material and applied to insulated pipes naturally the simplest way to 35 coil the jacketing material around the insulated pipe is in conformation to the curve of the material on the roll. The glass strand reinforcement has the warp threads running lengthwise of the roll. The dimensions of the sheet as formed is of course, continuous as to length, but it is 40 cut off in 34 ft. 6 in. lengths and the width is about 38 inches to form a roll of approximately 108 sq. ft. The reinforcing strands will be widthwise of the cut piece wrapped around the insulated pipe and the resistance to 45 tearing will be effective when the binding wires are wrapped around the pipe and the ends of the wires are clinched or twisted together.

50 The men installing the jacketing can make a more secure and snug wrap and clinching of the binding wires and weather resistance will be promoted. There is nothing 55 which will cause deterioration of an installation quicker than loose fitting of the jacketing material. Water gets in between the jacket and insulation with each rain and the effectiveness of the entire installation deteriorates rapidly. Thus the particular positioning of the fill threads in the composite web of jacketing material is more effective when it resists tearing of the edges of a piece cut to size to surround an insulated pipe.

Preferably the glass scrim which is combined in the web may be made as follows:

The product may be made from fiber yarns of various constructions fabricated to resemble conventional open mesh scrim fabrics, but differs in that the usual "over and under" weave is eliminated and the fabric pattern maintained by the use of an adhesive which "welds" the warp and fill together at each crossover point.

The physical properties of the glass scrim may be substantially as follows:

Average tensile strength (individual ends):

|      | Lbs. |
|------|------|
| Warp | 12.4 |
| Fill | 8.0  |

Nominal weight per 100 lineal yards:

Width: 36" \_\_\_\_\_ lbs. 3.39

Ignition loss—40%—10%.

Our product is a durable, weather-resistant jacketing specifically designed for the protection of outdoor insulated pipe lines where the danger of fire must be minimized. Ordinary roofing jackets are not satisfactory, because they burn, spread fire, and drip asphalt, which further contributes to combustion. Our product is recommended for use in the process industries and in oil refineries, where it affords maximum resistance to the spread of fire—and further protects the insulated surface from weather damage.

The product consists of a tough, substantial sheet of asphalt saturated asbestos felt, over which is cemented on one side an unsaturated asbestos sheet. The complete sheet is reinforced with a fabric of tough, flexible glass threads. This construction combines flexibility with very high tensile strength and extremely great resistance to tearing and cutting from wire or strap fastenings.

Our product should be applied with the white side out on all straight runs of pipe or expansion bends with at least 3 inch circumferential and lateral laps. On horizontal pipes, the laps should be located on the side of the pipe, turned downward. The jacket may be held securely in place with rings of No. 16 gauge copper weld wire or strapping on not greater than 4 to 6 inch centers.

As a test to determine the resistance to tearing or cutting of the outer covering of the jacket may be accurately determined by a machine which we have devised for determining these properties. We have diagrammatically illustrated such a machine in FIGURES 4 and 5 wherein:

FIGURE 4 is a fragmentary side elevational view of a tear resistance measuring apparatus.

FIGURE 5 is a fragmentary view showing a modified type of holder for the sheet of which the tear resistance is to be determined.

FIGURE 6 is a side elevation of fire testing apparatus for pipe jacketing.

A pair of metal plates 10 are hinged together as at 11 and one of the plates has an angular base 12 at its rear face by means of which it may be mounted on a wall as with screws 13. The plates are further connected with bolts 14 having nuts 15 by means of which the plates may be clamped together. Each of the plates has a slot 16 extending down from its top. A stud or post secures the end of a 16 gauge copper weld wire 17 similar to what with which the cylindrical pipe covering is to be subsequently wrapped.

On the other end of the wire there is secured a weight. Below the weight, which in this instance weighs 13.3 lbs., there is a pointer 18 which registers with a scale 19 subdivided to show inches and parts of inches or centimeters.

A piece of the multiply jacket material sheet 20 with the fill threads parallel with the top edge of the sheet is placed between the plates and clamped rigidly in position. The wire 17 is placed in the middle of the slots in the plates so as to freely contact the upper edge of the sheet to be tested. If the pointer begins to move down on the

scale the distance is measured and this indicates the relative tear resistance of the sheet to 16 gauge copper wire.

If the pointer 18 does not move down this indicates that the sheet is resisting the cutting force of the wire. Then another weight is placed on top of the 13.3 lb. weight. If no cutting takes place additional weights are added until the tearing begins.

With ordinary jacketing sheet material the resistance to tearing is practically nil. As an example, the wire 17

10 normally cuts down into the ordinary sheet 3 inches in 13 seconds. With our new multiply jacket sheet material with the 13.3 lb. weight on the tear strength gauge the arrow rarely moves down over 2 inches. It takes additional weights and a long period of time before the cut gets longer than 2 inches. We have adopted less than two inches tear in 24 hours as a standard for our product and it illustrates the surprising properties of our invention.

FIGURE 5 shows a modified type of paper clamp, 20 with the plates 10a secured together with thumb screws 14a and with the sheet to be tested clamped between the plates. This modification has an enlarged angular base 12a which supports the clamp on a horizontal support.

Other modifications of tear resistance gauges or devices 25 may readily be devised by those skilled in this art. As far as we are advised this measurement of tear resistance by a wire of similar dimensions to the wire normally used for binding the jacketing material in position is entirely new and we claim the same broadly herein.

The flame resistance testing of our new insulation outer covering product should be in accordance with the tests in the Federal specifications SS-A-118b, under sections 3.7; 3.7.1; 4.3.3 Table III, and the drawing of page 5 of said Federal specifications. Under such specified testing 30 our new material rates as class A flame resistant.

In order to test the efficacy of our product from the point of view of our first noted objective, i.e., covering for outdoor insulated pipe lines which will resist spread of flame and the dripping of asphalt which would otherwise propagate combustion, we have devised a testing apparatus as indicated in FIGURE 6.

This fire test for pipe jacketing material involves the suspension of the covered pipe suspended vertically. The larger area of the assembly is enclosed with a larger diameter pipe to form a flue and what we have called a "doughnut" burner to start the test. The test time is 10 minutes with the burner on throughout the test. At the end of this period the flue pipe is removed and the amount of flame spread and fire damage is determined.

Describing the apparatus there is an upper beam support 21 from which are suspended through a pulley 22, a plurality of cables 23 which are connected to the outer flue pipe 24. Thus the outer flue pipe may be elevated vertically to expose the pipe jacketing after the test is completed.

A two inch pipe 25 is independently suspended and the jacketing material, usually in segment, is secured on the pipe 25 in the usual manner. Then our new jacket covering material is wrapped around the insulated pipe, 60 the jacket covering material being secured to the pipe 25 with wire wraps spaced about four inches apart.

The length of the jacketed and covered pipe to be tested is six feet 9 1/4 inches. In position to carry out the test the jacketing and covering sheeting extends below the bottom of the outer flue pipe 24 about ten inches and the covered jacketing extends above the top of the flue pipe also about ten inches.

For testing our material there is a circular (doughnut type) heater 27 positioned about one inch below the bottom of the outer flue. This heater has a series of circumferentially arranged openings through which gas from a gas tube 28 is introduced.

With the various parts as described in assembled condition, the burner is lighted and the heat applied for ten minutes. At the end of this time the burner is

shut off, the outer flue is elevated and the extent of flame spread damage to the insulation outer jacket is determined by visual observation. Further the extent of splattering of asphalt dripping from the jacket is observed.

This test as has been described is primarily for purposes of comparison of different types of outer covering but with a standardization of the rate of flow of the gas to the burner as by passing the gas through a meter set to control the rate of flow and pressure. A test for different ratings of material all made in the same way may be 10 worked out, as will be readily understood.

Comparing insulating outer covering material made in accordance with the specifications set forth herein we have observed that our material shows very little burning. Competitive jacket covering material such as asphalt coated felt, similarly tested, shows the outer covering material practically consumed and charred away. At the same time the testing of our new material shows practically no dripping while competitive material shows an area of three or four feet covered with intermittent 20 splotches of drippings.

Modifications in the general plan of manufacture of the outer jacket covering material will occur to those skilled in the art, it being remembered that the substantial achieving of the six numbered objectives as set forth on page 1 25 of the specification will determine the extent of appropriation of our invention.

While we have explained that our invention relates to the outer covering material for insulation covered pipes, we have used the term jacketing as not including the insulative blocks or precast insulative segments, but only 30 the outer wrapping sheet which is usually wired in position.

Having thus described our invention, what we claim as new and desire to secure by Letters Patent is:

1. An outdoor, above ground, weather resistant jacket- 35 ing material for insulating pipes and the like, comprising

in combination a layer of asphalt saturated asbestos felt constituting the inner layer of said jacketing material, a coating of asphalt cement on said saturated layer, glass fibers embedded in said asphalt cement coating, and a layer of unsaturated asbestos felt adhered to said asphalt cement coating and forming the outer layer of said jacketing material, said outer layer incorporating a paraffin wax composition whereby said outer layer remains permanently white upon exposure to the weather, said material being formed in a roll, and said glass fibers being disposed with a substantial quantity of glass fiber threads lying parallel to the axis of said roll, whereby said jacketing material is highly resistant to cutting or tearing when wrapped around a pipe in the same sense in which said material is wound in the roll and secured by a plurality of wire ties, said parallel fibers serving to support said wire ties and resist cutting or tearing of said jacketing material.

2. Jacketing material according to claim 1 wherein said glass fibers are in the form of an unwoven scrim.

#### References Cited in the file of this patent

#### UNITED STATES PATENTS

|           |                         |                |
|-----------|-------------------------|----------------|
| 2,066,311 | Appel et al. -----      | Jan. 5, 1937   |
| 2,082,174 | Miller et al. -----     | June 1, 1937   |
| 2,311,572 | Reynolds -----          | Feb. 16, 1943  |
| 2,311,573 | Shoan -----             | Feb. 16, 1943  |
| 2,360,109 | Converse -----          | Oct. 10, 1944  |
| 2,523,022 | Horstman -----          | Sept. 19, 1950 |
| 2,620,851 | Brown -----             | Dec. 9, 1952   |
| 2,637,673 | Barnard -----           | May 5, 1953    |
| 2,706,909 | Boor -----              | Apr. 26, 1955  |
| 2,794,483 | Hopkins et al. -----    | June 4, 1957   |
| 2,828,798 | Hopkins et al. -----    | Apr. 1, 1958   |
| 2,897,841 | In Wai Hui et al. ----- | Aug. 4, 1959   |
| 2,943,010 | Stefi et al. -----      | June 28, 1960  |